

## UNITED STATES PATENT OFFICE

HERMANN VOIGTLÄNDER AND OTTO KAUFELS, OF ESSEN, GERMANY, ASSIGNEES TO  
FRIED. KRUPP AKTIENGESELLSCHAFT, OF ESSEN-ON-THE-RUHR, GERMANY

## PROCESS FOR PRODUCING ARTICLES OF REFRACTORY METAL ALLOYS

No Drawing. Application filed May 3, 1929, Serial No. 360,326, and in Germany May 2, 1928.

The invention has for its object a new process for the production of an alloy which consists of carbide of tungsten or molybdenum and of a lower melting metal or metalloid. This object is obtained according to the invention by melting down an alloy consisting of said refractory metals and of a lower melting metal or metalloid and carbon, and by pulverizing and sintering the mass.

10 The process may be performed e. g. in the following manner:

In a carbon or graphite resistance furnace an alloy is melted down containing at least 80 per cent of tungsten, at most 20 per cent 15 of a lower melting metal or metalloid (e. g. nickel, chromium, cobalt, iron, or silicon) and carbon. After solidification this alloy is pulverized as finely as possible and shaped to pressed bodies which are finally subjected 20 to a sintering process that intimately unites the particles of the bodies. The temperature required for the sintering operation lies at about 2200 to 2400 degrees C. The sintered alloy produced in this manner is remarkable 25 when compared with a cast alloy of the same composition for its greater ability to withstand the shocks to which tools are unavoidably exposed. In comparison with an alloy of the same composition but obtained by sintering a mixture of carbide of tungsten or 30 molybdenum and of a lower melting auxiliary metal the present alloy possesses the advantage, especially important for tools, that the finished alloy resists a much higher heat- 35 ing than the former.

We claim:

1. The process of producing articles of refractory metal alloys, which comprises melting together a refractory metal, a metal or 40 metalloid having a lower melting point, and carbon; allowing the fused mass to solidify; pulverizing the solidified mass, pressing the powder so produced into a body of any desired shape, and then sintering the body.
- 45 2. The process of producing articles of refractory metal alloys, which comprises melting together one of the metals tungsten or molybdenum, a metal or metalloid having a lower melting point and carbon; allowing 50 the fused mass to solidify; pulverizing the

solidified mass, pressing the powder so produced into a body of any desired shape, and then sintering the body.

The foregoing specification signed at Cologne, Germany, this 18th day of April, 55 1929.

HERMANN VOIGTLÄNDER.  
OTTO KAUFELS.

60

65

70

75

80

85

90

95

100